

Patented Nov. 3, 1936

2,059,208

# UNITED STATES PATENT OFFICE

2,059,208

## FIRE KINDLER

Franklin V. Chaney, New York, N. Y., assignor,  
by mesne assignments, to Pine Kindler Corporation,  
New York, N. Y., a corporation of Delaware

No Drawing. Application November 13, 1934,  
Serial No. 752,831

10 Claims. (Cl. 44—41)

This invention relates to fire kindlers and provides novel types of kindlers which are efficient, economical, odorless and clean to handle.

Fire kindlers of many types and kinds have 5 been devised heretofore which in general consist of a mixture of two or more of a wide variety of materials, but all such kindlers have been lacking in certain essential or desirable kindler characteristics, particularly in the ability to 10 quickly start an anthracite coal fire with the consumption of a comparatively small quantity of kindler. This is due to the fact that no one heretofore has been successful in producing fire kindlers having a heat unit content which is 15 sufficiently great so that small quantities thereof will provide economical means for quickly starting hard coal fires.

To increase the heat producing qualities of kindler materials, such as wood, attempts have 20 been made heretofore to saturate the wood by the open tank process with various combustible liquids, but such attempts have failed to increase materially the heat unit content of the wood because little, if any, saturation was effected. 25 This results from the fact that the constituent cells of the wood are filled substantially with sap which remains even after the wood has been seasoned. Accordingly, since the cells of the wood are filled, they are incapable of absorbing any 30 substantial quantity of other materials, in consequence of which the heat unit content of the wood after such efforts to saturate it, remained approximately at the heat unit content of the natural wood with its sap content.

35 The present invention provides fire kindlers which possess such high heat producing qualities that the burning of small quantities thereof will quickly start anthracite coal fires and other fires, including bituminous coal, coke, wood, etc. The 40 kindlers of my invention are additionally readily ignited by contact with flame and are clean and convenient to handle.

The nature of the invention will be understood clearly from the following description.

45 Generically, my kindlers have a base material of fibro-cellular character, the cells of which previously have been emptied or substantially emptied of the material with which they normally are filled during growth or development. This 50 extracted base material is saturated or impregnated thoroughly with inflammable material or a mixture of inflammable materials of desirable burning and heat producing characteristics until the impregnating material substantially fills the 55 emptied cells. Preferably, the impregnated base material also is coated with inflammable material having a melting point above ordinary temperatures in order to maintain and increase the heat unit content of the kindlers by preventing 60 any substantial evaporation of the impregnating

material and to render the kindlers odorless and make them clean to handle.

The base material for the kindlers may be any desired form of fibro-cellular material of vegetable origin, from which the sap content has 5 been removed entirely or for the major part from the constituent cells. Methods by which the sap content of such fibro-cellular materials may be extracted are well known and need not be described here since they form no part of my 10 invention. Ordinarily, the extraction of the sap content of these materials, is effected after the materials have been reduced by suitable known means to relatively finely divided form, such as small particles, or chips, or constituent fibers or 15 groups of fibers. The extraction of the sap content from the cells of these materials leaves them in a condition in which they will readily absorb volumes or quantities of inflammable materials of high B. t. u. content much greater than 20 the volume of the extracted base material, so that upon combustion in small quantities, the impregnated base material will produce heat in sufficient quantity and intensity to readily ignite anthracite coal fires for all purposes, as well as 25 bituminous coal, coke, wood and other fires. I believe that I am the first to discover the great advantage which accrues from the use for kindler purposes, of vegetable fibrous material 30 from which the sap content has been extracted. 80

The preferred base material is extracted wood, which has been finely divided into small particles or chips or into separated or partly separated fibers of the wood. It will be understood however, that I do not limit myself to extracted wood, 35 since other extracted fibro-cellular materials of vegetable origin are effective for this purpose. Among them may be mentioned, sugar cane, bagasse and corn stalks.

The inflammable material or materials utilized 40 for impregnating the extracted vegetable fibro-cellular materials may be of any suitable character. Hydrocarbon-containing materials, including crude petroleums, fuel oils, by-products in the production of waxes and oils of various 45 kinds and many asphalt and coal tar products may be used. It will be understood that these particular materials are enumerated merely as examples of suitable impregnating materials and that I do not wish to be limited thereto. In the 50 selection of inflammable materials for impregnating the extracted base material, it is desirable to use some material of a quickly inflammable nature and some material of a slow burning nature. The choice of the particular material or 55 materials for impregnation will be governed by the quantity and intensity of heat it is desired to produce upon combustion of the kindler.

Various coating materials may be used for the 60 impregnated base material, but I prefer that a

material or mixture of materials be used which has a melting point well above ordinary temperatures so that it may be applied in a liquid condition and upon cooling, will become and remain 5 hard and solid at ordinary temperatures so that the kindlers will not be "tacky" or objectionable to handle. Rosin, lacquer and some qualities of varnish are suitable for this purpose. The coating material may be applied after the impregnated 10 base material has been formed into kindler blocks or it may be mixed with the impregnating materials before they are brought into contact with the base material. The preferred coating material is limed rosin which consists of a mixture 15 of rosin having a melting point of about 125 degrees to 150 degrees F. and 3% to 5% of lime, by weight. The point at which this material softens or becomes "tacky" is normally between 175 degrees to 200 degrees F. I believe I am the first to discover the effectiveness of limed rosin 20 and rosins having relatively high melting points as coating materials for fire kindlers.

A preferred method of producing fire kindlers of preferred composition which embody my invention, is as follows: Pine wood chips from 25 which the sap content has been extracted and varying in length from about one-half inch to about one inch and preferably about one-eighth inch in breadth or thickness, are first thoroughly 30 dried until the water content does not exceed five to eight percent. These dried chips are introduced into a suitable mixing tank provided with means, such as steam coils, for heating, and equipped with suitable agitating apparatus. If 35 desired, the chips may be dried in the mixing tank. To the chips in the mixing tank there is added uncracked fuel oil of high B. t. u. content, preferably about 18,000 to 19,000 B. t. u.'s per pound, to about 10% of the weight of the dry 40 chips. This mixture is agitated for a period of about one hour or until the dry chips have absorbed the fuel oil. Thereafter, asphalt of the grade known as "N. J. 110", or its equivalent such as coal tar, is added to the impregnated chips 45 in the mixing tank, in a quantity approximating 70% of the chips by weight. This mixture is agitated for a period of from one to two hours, or for such time as may be required for the asphalt to be absorbed or taken up by the chips. This 50 "N. J. 110" asphalt is relatively slow burning; it burns with little or no residue; has a heat value of about 20,000 B. t. u.'s per pound and in addition to increasing greatly the heat content of the chips, also provides a binder therefor. 55 Next, there is added melted limed rosin to about 20% of the weight of the chips, this rosin preferably having a lime content of 3% to 5% of the rosin by weight, to increase its melting or "tacky" point to within the range between 175 degrees 60 and 200 degrees F. This limed rosin has a heat value of about 15,000 B. t. u.'s per pound. The impregnated chips and limed rosin are agitated for a short period of time, about one-quarter to one-half an hour, until the chips are coated. 65 Thus the chips absorb at least 100% by weight of hydrocarbon-containing inflammable material.

The mixing and agitation of the extracted chips with the asphalt, fuel oil and limed rosin is preferably carried out at a temperature of 70 about 200 degrees F. With this method the chips will absorb practically all of the liquid mixture and thereby will become impregnated thoroughly with the inflammable material. Thereafter the impregnated and coated chips are formed into 75 kindler blocks of any desired dimensions by any

suitable means, such as moulding, pressing or the like. Upon cooling, the kindlers will retain their shape and will have a hard exterior which will not be unpleasant to handle.

If desired, the dry extracted chips may be 5 impregnated in the mixing tank as above described but without the rosin content of the mixture, then formed into kindlers and thereafter suitably coated with melted limed rosin, preferably maintained at a temperature of about 350 10 degrees F.

If desired, the dry chips may be impregnated in the manner aforesaid, or in any other convenient manner, with fuel oil, asphalt and ordinary 15 rosin and after the mixture is formed into kindler blocks and cooled to about 100 degrees F., the blocks may be coated with limed or high melting point rosin. In this case only a very thin rosin coating is necessary and if applied by immersing the kindler blocks in a bath of the rosin, the bath 20 should be maintained preferably at a temperature of about 350 degrees F. to insure a suitably thin coating.

If a fire kindler having quicker ignitability 25 and faster burning characteristics is desired, about 10% by weight of crude naphthalene may be added to the extracted chips in the mixing tank. I have found, however, that naphthalene is not required for ordinary fire lighting purposes.

A method of producing a kindler embodying my 30 invention and having a base material of fibrated vegetable fibro-cellular material from which the sap content has been extracted, or of such material reduced to fibers or groups of fibers, is as follows: Extracted pine wood chips which have 35 been sufficiently finely divided are thereafter reduced by suitable means to their constituent fibers or groups of fibers. These separated fibers or fiber groups are then formed into boards of suitable thickness and are thereafter cut into 40 blocks of desired length and breadth for fire kindler purposes. Desirable dimensions for this purpose are approximately 6" long, 3" wide and  $\frac{3}{4}$ " thick. An impregnating mixture of about 45 60% fuel oil of high B. t. u. content and 30% of the aforementioned "N. J. 110" asphalt, or its equivalent such as coal tar to which there is added preferably 10% crude naphthalene, is placed in a suitable receptacle which may be heated and maintained at a temperature 50 of about 200 degrees F. The blocks of base material are introduced into this mixture by suitable means and allowed to remain for a short time, about five to ten seconds, during 55 which they will absorb 150 to 200% of their own weight of the mixture. Thereafter, the blocks are removed and permitted to cool to a temperature of about 100 degrees F. or less. The cooled blocks are then passed as rapidly as possible 60 mechanically through a bath of melted limed rosin maintained at a temperature of about 350 degrees F. Immersion of the blocks in the limed rosin for from one to three seconds will be sufficient to adequately coat the blocks. Thereafter the blocks are removed and the rosin coating immediately hardens which provides the kindlers with a clean, hard coating.

It will be perceived that fire kindlers embodying my invention will possess enormous heat 70 producing qualities, which are sufficient to start anthracite coal fires and other fires more quickly than can be done with charcoal or kindling wood and at a cost which is less than that for charcoal, on a heat unit content basis.

It will be evident that wide variations are possible in the composition of fire kindlers embodying my invention without transcending the invention. Any desired fibro-cellular material of vegetable origin from which the content of the cellular structure of the material has been extracted to the extent desired, may be employed. The greater the degree of extraction of the sap content, the greater will be the degree of absorption of, or impregnation with, inflammable material and the greater will be the heat producing potentialities of the kindler. The size of the particles, chips, fibers or fiber groups may be varied as desired within limits. Preferably, these should be such that when the kindler is formed, a sufficient number of interstices remain between the particles, chips or fibres to impart a porous character to the kindler so that when ignited, air will reach the interior portions and these will be burned at the same time the exterior portions of the kindler are burned. Complete burning thus will be effected with the production of great heat.

Tests conducted at the Anthracite Institute Laboratory of Primos, Pa., which is the official testing station of practically all of the coal interests of the United States, were made on fire kindlers embodying my invention as compared with charcoal, which product is regarded as being more efficient than ordinary kindling wood, and these tests conclusively demonstrated the superiority of my fire kindlers as compared with charcoal in the lighting of anthracite coal fires. These tests were made under identical conditions. The cost to the consumer of kindling material used in the tests was the same in all three instances. As measured by cost, an equal amount of my extracted wood chip kindler and my extracted wood fibre kindler and ordinary charcoal was used, together with the same quantities of the same anthracite coal for each fire built and all other conditions were exactly the same with the single exception that the full charge of coal was placed on top of my kindlers before the same were lighted whereas in the case of the charcoal kindled fire, no coal was placed on top of the charcoal until the same had been burning for a period of seven to eight minutes, after which time the coal was added.

Complete ignition of the coal was obtained with both the chip kindler and the fibre kindler in less than half the time required for complete ignition of the coal by the charcoal kindled fire. Accordingly, it will be clear that kindlers embodying my invention are more efficient and economical to use and produce a faster fire than either charcoal or kindling wood and with less labor involved.

To effect greater economy in the manufacture of fire kindlers embodying my invention, waste extracted wood chips may be utilized, large quantities of which are made available as a result of sap extraction processes carried out to obtain turpentine and pitch.

I desire it to be understood that I entertain no intention to limit the present invention, except by the scope of the appended claims.

What I claim is:

1. A fire kindler consisting essentially of relatively finely divided, uncharred particles of vegetable fibro-cellular material free from sap, containing by absorption at least 100% by weight of a hydrocarbon-containing inflammable material selected from the group consisting of crude petroleum, fuel oil, asphalt and coal tar.

2. A fire kindler consisting essentially of relatively finely divided, uncharred particles of vegetable fibro-cellular material free from sap, containing by absorption at least 100% by weight of a hydrocarbon-containing inflammable material selected from the group consisting of crude petroleum, fuel oil, asphalt and coal tar, and coated with an inflammable material which is non-tacky at ordinary temperatures. 5

3. A fire kindler consisting essentially of relatively finely divided, uncharred particles of vegetable fibro-cellular material free from sap, containing by absorption at least 100% by weight of a mixture of fuel oil, asphalt and naphthalene, the naphthalene being a minor proportion of 15 the mixture. 10

4. A fire kindler consisting essentially of relatively finely divided, uncharred particles of vegetable fibro-cellular material free from sap, containing by absorption at least 100% by weight of fuel oil, asphalt and rosin, the rosin being a minor proportion of the mixture. 20

5. A fire kindler consisting essentially of relatively finely divided, uncharred particles of vegetable fibro-cellular material free from sap, containing by absorption at least 100% by weight of a mixture of fuel oil, asphalt and naphthalene, the naphthalene being a minor proportion of the mixture, and coated with an inflammable material which is non-tacky at ordinary temperatures. 25 30

6. A fire kindler consisting essentially of relatively finely divided, uncharred particles of vegetable fibro-cellular material free from sap, containing by absorption at least 100% by weight of fuel oil, asphalt and rosin, the rosin being a minor proportion of the mixture, and coated with an inflammable material which is non-tacky at ordinary temperatures. 35

7. A fire kindler consisting essentially of relatively finely divided, uncharred particles of wood, all of the sap content of which has been removed prior to the use of such material for fire kindlers, containing by absorption at least 100% by weight of a mixture of fuel oil, asphalt and naphthalene, the naphthalene being a minor proportion of the mixture. 40 45

8. A fire kindler consisting essentially of relatively finely divided, uncharred particles of wood, all of the sap content of which has been removed prior to the use of such material for fire kindlers, containing by absorption at least 100% by weight of a mixture of fuel oil, asphalt and rosin, the rosin being a minor proportion of the mixture. 50

9. A fire kindler consisting essentially of relatively finely divided, uncharred particles of wood, all of the sap content of which has been removed prior to the use of such material for fire kindlers, containing by absorption at least 100% by weight of a mixture of fuel oil, asphalt and naphthalene, the naphthalene being a minor proportion of the mixture, and coated with an inflammable material which is non-tacky at ordinary temperatures. 55 60

10. A fire kindler consisting essentially of relatively finely divided, uncharred particles of wood, all of the sap content of which has been removed prior to the use of such material for fire kindlers, containing by absorption at least 100% by weight of a mixture of fuel oil, asphalt and rosin, the rosin being a minor proportion of the mixture, and coated with an inflammable material which is non-tacky at ordinary temperatures. 65 70

FRANKLIN V. CHANEY.